

## UNITED STATES PATENT OFFICE

2,096,607

## MANUFACTURE OF ARTIFICIAL YARN, FILAMENTS AND THE LIKE

Thomas H. Byron, Elizabethton, Tenn., assignor to North American Rayon Corporation, New York, N. Y., a corporation of Delaware

No Drawing. Application October 25, 1934,  
Serial No. 749,923

8 Claims. (Cl. 106—40)

My present invention has to do with a new and novel way of producing colored and delustrated yarn.

In the manufacture of yarn from cellulosic solutions, it is old to add an insoluble pigment to the spinning solution prior to its extrusion to form fibres, filaments, yarn, and the like. For example, the Singmaster U. S. Patent 1,725,742 broadly covers the idea of adding an insoluble pigment to yarns in order to delustre them, while a later Singmaster U. S. Patent 1,875,894 refers specifically to the use of titanium dioxide for this purpose. These added compounds tend to reduce the lustre of the yarn, and produce so-called low lustre products.

The tinting of yarn, per se, is also an old expedient, and Lockhart's U. S. Patent 1,865,701, for example, indicates that by including colored matter in the solution a dyed or colored yarn can be directly produced.

Both of the class of patents just described fulfill their individual functions in a satisfactory manner, but my present invention differs from, and is an improvement over these, in that a single compound only is added to the spinning solution in order to produce the double result of both delustring and coloring the resulting yarn. The importance of this innovation becomes readily apparent when one considers that great difficulties with respect to filtering and spinneret clogging present themselves when any matter is added to a spinning solution.

As a further differentiation, it may be pointed out that in my present invention it is not absolutely necessary that the salt added to the viscose, cuprammonium, or other cellulosic solution, be insoluble therein, or impervious to the action of acids and bases.

My present invention concerns the use of titanates and metatitanates as ingredients which not only delustre but also color the yarn produced from the solutions containing these salts.

In the viscose and cuprammonium processes, a small amount varying from 0.4 to 4.5% (calculated on the cellulose content) of the titanate or metatitanate may be finely ground in the customary manner and thoroughly mixed with the solution. In the production of nitrocellulose and organic derivatives of cellulose solutions, the salts may be mixed with either the cellulose per se, the finished solution, or the solvent, in the amounts previously indicated.

As an example I may make use of cobalt titanate or cobalt metatitanate, ordinarily produced by mixing cobalt carbonate with titanium dioxide,

and calcining. A bright green color is imparted to the threads produced, and their lustre is also diminished. By controlling the calcining temperature various shades of green may be produced.

Vanadium titanates may be employed if an orange-yellow color, or one approaching that, is desired. Similarly, iron, nickel, chromium, and other salts may be used to replace the cobalt and thus a variety of colors are available.

The salts need not be totally or partially insoluble in the solutions, or in the following treating media, since, according to one theory, the titanium salts present tend to produce the oxide which acts as a delustrant. If the salt used is totally impervious to the solution and treating media employed, the whole salt will act as an ordinary insoluble pigment, and both color and delustre the yarn.

In the claims I wish to have the term titanate include also the so-called metatitanate salts.

Having now set forth my invention as required by the patent statutes, what I desire to claim is:

1. A spinning solution for the manufacture of cellulosic products comprising a cellulosic solution selected from the group consisting of viscose and cuprammonium cellulose containing a finely divided titanate selected from the group consisting of cobalt, chromium, iron, nickel and vanadium titanates in a sufficient amount to color and simultaneously deluster the products formed from said solution.

2. A spinning solution for the manufacture of cellulosic products comprising a cellulosic solution selected from the group consisting of viscose and cuprammonium cellulose containing a finely divided cobalt titanate in a sufficient amount to color and simultaneously deluster the products formed from said solution.

3. A spinning solution for the manufacture of cellulosic products comprising a cellulosic solution selected from the group consisting of viscose and cuprammonium cellulose containing a finely divided chromium titanate in a sufficient amount to color and simultaneously deluster the products formed from said solution.

4. A spinning solution for the manufacture of cellulosic products comprising a cellulosic solution selected from the group consisting of viscose and cuprammonium cellulose containing a finely divided vanadium titanate in a sufficient amount to color and simultaneously deluster the products formed from said solution.

5. Regenerated cellulose of the group consisting of viscose and cuprammonium cellulose con-

taining a finely divided titanate selected from the group consisting of cobalt, chromium, iron, nickel and vanadium titanates, said titanate being present in a sufficient amount to color and simultaneously deluster said cellulose.

6. Regenerated cellulose of the group consisting of viscose and cuprammonium cellulose containing a finely divided cobalt titanate, said titanate being present in a sufficient amount to color and simultaneously deluster said cellulose.

7. Regenerated cellulose of the group consisting

of viscose and cuprammonium cellulose containing a finely divided chromium titanate, said titanate being present in a sufficient amount to color and simultaneously deluster said cellulose.

8. Regenerated cellulose of the group consisting of viscose and cuprammonium cellulose containing a finely divided vanadium titanate, said titanate being present in a sufficient amount to color and simultaneously deluster said cellulose.

5

10

THOMAS H. BYRON.